

# United States Patent Office

2,830,017

Patented Apr. 8, 1958

1

2,830,017

## METHOD OF FORMING A SACRIFICIAL LUBRICATING LAYER

James J. Shyne, Arlington, and Frederick Fahnoe, Morris-town, N. J., assignors to Vitro Corporation of America, Verona, N. J.

No Drawing. Application January 18, 1954  
Serial No. 404,796

4 Claims. (Cl. 204—181)

Our invention relates to a method of producing lubricated metal structures.

In many conventional metal working processes such as drawing, shaping, forming, threading, extruding and the like, it is often necessary to lubricate the metal structure to be so treated either before or during the working operation. Therefore, a coating composed of solid or liquid lubricants is generally applied to the structure by brushing, spraying, dipping or other conventional techniques. As far as is known to us, such coatings are characterized by variable thickness, poor adherence to the metal, and, in certain situations, inadequate lubricating and anti-seizing properties.

Accordingly, it is an object of the present invention both to provide a metal structure having a lubricant coating which obviates the above disadvantages and a novel method for applying this coating.

Another object is to provide a metal structure having a lubricant coating which will adhere well to the structure until the desired metal working operation is performed and which can be readily stripped from the structure during this operation.

Still another object is to provide a method for electrophoretically depositing a solid lubricant coating on a metal structure.

Yet another object is to provide a metal structure having a lubricant coating with excellent lubricating and anti-seizing properties.

Still a further object is to provide a lubricant coating which will reduce the coefficient of friction of metals possessing adhesive properties as well as those metals which cannot be surface hardened.

Our invention contemplates the electrophoretic co-deposition of reducible or decomposable metallic compounds and laminated metallic lubricating agents on a metal structure of the character indicated and the subsequent reduction or decomposition of metal of the deposited reducible compound to form a metal matrix which is bonded to the structure and which in turn entraps and bonds the lubricating agent or agents to the structure to form a lubricant coating. The amounts of lubricant and matrix forming material are such that the layer after reduction contains 70-80% by weight of metallic matrix and 30-20% of solid lubricant. The relative proportions of the reducible compounds and lubricating agents are such that the lubricant coating will adhere uniformly to the structure until the structure is subjected to a metal working operation such as deep drawing. During this operation, the coating, while supplying the desired amount of lubrication, is progressively worn away or stripped from the structure. The term "sacrificial layer" has been selected to denote this type of coating and this term will be used hereinafter.

Certain inorganic compounds of metals and non-metals, for example, the sulphides, disulphides, selenides, and tellurides of such metals as molybdenum, tungsten, titanium, and uranium are characterized by a laminated or plate-like crystal structure in which the metallic atoms are attached to each other in a single common plane, while the non-metallic atoms are attached to the me-

2

tallic atoms to form layers on both sides of this plane. The non-metallic atoms in each of the several crystals thus formed have very little attraction for each other, so that these crystals will slip readily with respect to each other under the action of low shearing forces. Moreover, the non-metallic atoms have an affinity for adjacent metal surfaces, so that the crystals attached to such surfaces will exhibit very strong resistance to the action of forces normal to the direction of sheer. Consequently, these compounds have excellent lubricating properties and also have excellent anti-seizing properties. The term "laminated metallic lubricating agents" has been selected to denote compounds of this class and this term will be used hereinafter.

15 Electrophoretic deposition occurs when an electrostatic field is established between two electrodes immersed within a colloidal or gross dispersion of charged particles, thus causing migration of the suspended particles toward one of the electrodes and producing the deposit of an adherent coating on that electrode. Exceptional uniformity of coating thickness and compacting (with an attendant relatively high coating density) are obtained as compared with dipping, spraying, brushing and other conventional methods of application. Irregularly shaped objects can be coated with excellent uniformity and reproducibility of coating. A complete description of the electrophoretic process will be found in our copending application S. N. 386,882 filed October 19, 1953.

In another copending application S. N. 402,402, filed 30 January 5, 1954, we disclosed a method for electrophoretically forming a friction element on a base member; the element so formed comprises a metal matrix well bonded to the base member and a friction modifying agent entrapped within the interstices of this matrix. 35 The resulting device is characterized by a very strong element-member bond and by long wearing surface properties of the element. While this method is quite similar to that used in the present application, in contradistinction, the present invention discloses a metal structure 40 provided with a sacrificial layer and characterized by a weak layer-structure bond and by a lubricating surface which wears away rapidly.

The following examples set forth certain well defined instances of the application of this invention. They are, 45 however, not to be considered as limitations thereof, since many modifications can be made without departing from the spirit and scope of this invention.

### Example I

50 A gross dispersion containing 75% by weight of nickel oxide particles and 25% by weight of molybdenum disulphide was immersed in isopropyl alcohol and diluted to a 5% concentration in the manner outlined in the above mentioned copending application, S. N. 386,882.

55 This dispersion was then poured into a conventional electrophoretic bath. A one inch by four inch type 304 stainless steel panel was suspended in the dispersion and connected as the cathode. A steel plate was suspended in the dispersion and connected as the anode. The plate panel separation was adjusted to 3 inches and a direct voltage of 500 volts was applied between the anode and cathode. Nickel oxide and molybdenum disulphide particles immediately began to codeposit on one surface of the panel. After a 5 to 10 second interval, the panel 60 was disconnected and removed from the bath. The co-deposited coating attained a thickness of from 1 to 10 microns during this interval.

65 The panel was then fired in the atmosphere of hydrogen at a temperature of 1400° F. for a period of 15 seconds. Subsequent cross-sectional analysis established that the nickel oxide was reduced to nickel in the form of a matrix bonded by codiffusion to the surface of the

panel. The molybdenum disulphide particles did not enter into the reaction as the presence of hydrogen prevented oxidation, but were entrapped within the pores or interstices of the nickel matrix. The ratio by weight of nickel to molybdenum disulphide was found to be approximately 3 to 1.

The nickel-steel bond was found to be sufficiently strong to prevent damage to the coating during normal manual handling; however, the coating could be scratched away by any sharp pointed metal object.

The coated panel was inserted into a metal forming punch and die fixture and a one-half inch diameter section of the panel was drawn to a depth of  $\frac{1}{2}$ ". An uncoated type 304 stainless steel panel of the same dimensions was similarly tested and could not be drawn to a depth greater than  $\frac{1}{8}$ " without breaking.

The above process was repeated with different weight percentages of nickel oxide and molybdenum disulphide. When the percentage by weight of the disulphide was increased appreciably beyond 30%, the resultant coating did not adhere well to the panel; when this percentage was reduced appreciably below 20%, the lubricating properties were not satisfactory. Best results were obtained by holding the percentage by weight of molybdenum disulphide within the range 22-29%.

It was found that the firing temperature within the range 1300-1800° F. was satisfactory.

#### Example II

A coating 1 to 10 microns thick containing 77% by weight of nickel oxide and 23% by weight of molybdenum telluride was electrophoretically deposited on a segment of molybdenum wire in the same general manner as described above. The coated wire was then fired in a hydrogen atmosphere at a temperature of 1400-1600° F. for a period of 15 to 25 seconds.

Wire drawing operations were then performed on this coated wire and a like segment of uncoated wire. It was found that the allowable cross-sectional area reduction for a single draw of the coated segment was approximately twice as large as that obtained with the uncoated segment.

The above process was repeated with different weight percentages and with different firing temperatures and the results were substantially the same as in Example I.

#### Example III

A coating containing 78% by weight of silver oxide particles and 22% by weight of molybdenum disulphide particles was electrophoretically deposited on a titanium sheet in the manner outlined in Example I.

The coated sheet was then fired in helium at a temperature of from 1200 to 1400° F. for a period of 15 to 25 seconds. Subsequent cross-sectional analysis established that the silver oxide had been decomposed to silver in the form of a matrix bonded by codiffusion to the surface of the sheet. The molybdenum disulphide particles were entrapped within the pores of the silver matrix. The ratio by weight of silver to molybdenum disulphide was found to be approximately 3 to 1. The amount of silver oxide used to form the matrix may, however, be between 70 and 80% by weight and the corresponding amount of molybdenum disulphide between 30 and 20% by weight.

A titanium sheet with a sacrificial layer prepared in this manner was subjected to the drawing operation described in Example I. The coated sheet was successfully drawn to a depth of  $\frac{1}{2}$ ". An uncoated titanium sheet was similarly tested and could not be drawn to a depth greater than  $\frac{1}{8}$ " without breaking.

Many other materials can be used instead of those disclosed in the working examples. For example, the reducible or decomposable compounds can be oxides, hydrides or decomposable salts of such metals as copper, tin, zinc, chromium and various combinations of these

oxides as well as the oxides, hydrides and salts of nickel and silver. The metallic structure can be formed for example, from zirconium, beryllium and various alloys of these metals as well as steel, titanium and copper alloys.

Although in the above examples we have indicated certain definite firing temperatures, duration of reactions, etc., it is to be understood that any or all of these can be varied widely within the scope of our invention, since the particular conditions of operation are governed largely by the specific end structure desired. For example, the firing temperature must be high enough to perform the desired reduction of decomposition and low enough to prevent softening or melting of the materials used. The actual temperature will vary depending on the characteristics of these materials.

If necessary, that portion of the sacrificial coating which may adhere to the metal structure after the forming operation can be removed either manually or by chemical means such as pickling in selective agents.

Therefore, it is apparent that many widely different embodiments of this invention can be made without departing from the spirit and scope thereof and we do not intend to be limited except as indicated in the appended claims.

We claim:

1. The method of forming a sacrificial lubricating layer upon a selected surface of a metallic structure, said method comprising the steps of electrophoretically codepositing a mixture of a metallic matrix forming material of the group consisting of silver oxide and nickel oxide and a solid lubricant of the group consisting of the sulfides, disulfides, selenides and tellurides of molybdenum, out of a liquid organic medium upon said surface, the amounts of said matrix forming material and solid lubricant producing a layer having 70-80% by weight of metallic matrix and 30-20% of solid lubricant, and heating said structure in a gaseous atmosphere at a temperature to reduce said matrix forming material to form a metallic matrix which is bonded to said surface of said metallic structure, and which entraps and bonds said lubricant to said metallic structure.

2. The method of claim 1 in which the matrix forming material is nickel oxide, the lubricant is molybdenum disulfide, and the structure is heated in a hydrogen atmosphere at a temperature falling within the range 1300-1800° F. to reduce said nickel oxide to nickel.

3. The method of claim 1 in which the matrix forming material is nickel oxide, the lubricant is molybdenum telluride and the structure is heated in a hydrogen atmosphere at a temperature falling within the range 1400-1600° F. to reduce said nickel oxide to nickel.

4. The method of forming a sacrificial lubricating layer upon a selected surface of a titanium structure, said method comprising the steps of electrophoretically codepositing between 70 and 80% by weight of silver oxide and between 30 and 20% by weight of molybdenum disulphide out of a liquid organic media upon said surface; and heating said structure in an atmosphere of inert gas to a temperature falling within the range 1200 to 1400° F. for a period sufficient to decompose said silver oxide to silver whereby said layer is formed.

#### References Cited in the file of this patent

#### UNITED STATES PATENTS

|              |                      |               |
|--------------|----------------------|---------------|
| 2,202,054    | Hensel et al. -----  | May 28, 1940  |
| 2,488,731    | Lambert et al. ----- | Nov. 22, 1949 |
| 2,530,546    | Snyder -----         | Nov. 21, 1950 |
| 2,576,362    | Rimbach -----        | Nov. 27, 1951 |
| 70 2,640,024 | Palmaeir -----       | May 26, 1953  |
| 2,650,975    | Dorst -----          | Sept. 1, 1953 |
| 2,708,726    | Atherton -----       | May 17, 1955  |

#### FOREIGN PATENTS

|              |              |               |
|--------------|--------------|---------------|
| 75 1,044,212 | France ----- | June 17, 1953 |
|--------------|--------------|---------------|